

[54] **HEXACHLOROCYCLOPENTENE  
CHEMICAL SENSITIZERS FOR  
HETEROGENEOUS ORGANIC  
PHOTOCONDUCTIVE COMPOSITIONS**

[75] **Inventor:** William E. Yoerger, Rochester, N.Y.

[73] **Assignee:** Eastman Kodak Company,  
Rochester, N.Y.

[21] **Appl. No.:** 800,483

[22] **Filed:** May 25, 1977

[51] **Int. Cl.<sup>2</sup>** ..... G03G 5/04

[52] **U.S. Cl.** ..... 96/1.5 R; 260/648 C;  
96/1.6; 252/501

[58] **Field of Search** ..... 96/1.6, 1.5; 260/648 C

[56] **References Cited**

**U.S. PATENT DOCUMENTS**

3,349,064 10/1967 Gumboldt et al. ..... 526/143

**OTHER PUBLICATIONS**

Chemical Abstracts, vol. 66, col. 33526s.

*Primary Examiner*—John D. Welsh  
*Attorney, Agent, or Firm*—T. N. Dahl

[57] **ABSTRACT**

Photoconductive insulating compositions in the form of organic photoconductive dispersions are described. Particles of organic photoconductor such as p-terphenyl are dispersed in cellulose nitrate and chemically sensitized with monomeric hexachlorocyclopentenes to provide useful heterogeneous photoconductive insulating dispersions. Such dispersions can be applied to an electrically conducting support to prepare electrophotographic elements.

**16 Claims, No Drawings**

HEXACHLOROCYCLOPENTENE CHEMICAL  
SENSITIZERS FOR HETEROGENEOUS ORGANIC  
PHOTOCONDUCTIVE COMPOSITIONS

BACKGROUND OF THE INVENTION

1. Field of the Invention

This invention relates to electrophotography and particularly to chemical sensitization of heterogeneous photoconductive compositions and electrophotographic elements with highly chlorinated monomeric chemical sensitizers.

2. Discussion of Related Art

The process of xerography, as disclosed by Carlson in U.S. Pat. No. 2,297,691 (issued Oct. 6, 1942), employs an electrophotographic element comprising a support material bearing a coating of a normally insulating material whose electrical resistance varies with the amount of incident electromagnetic radiation it receives during an imagewise exposure. The element, commonly termed a photoconductive element, is first given a uniform surface charge, generally in the dark after a suitable period of dark adaptation. It is then exposed to a pattern of actinic radiation which has the effect of differentially reducing the potential of this surface charge in accordance with the relative energy contained in various parts of the radiation pattern. The differential surface charge or electrostatic latent image remaining on the electrophotographic element is then made visible by contacting the surface with a suitable electroscopic marking material. Such marking material or toner whether contained in an insulating liquid or on a dry carrier, can be deposited on the exposed surface in accordance with either the charge pattern or discharge pattern as desired. Deposited marking material can then be either permanently fixed to the surface of the sensitive element by known means such as heat, pressure, solvent vapor, or the like, or transferred to a second element to which it can similarly be fixed. Likewise, the electrostatic latent image can be transferred to a second element and developed there.

Various photoconductive insulating materials have been employed in the manufacture of electrophotographic elements. For example, vapors of selenium and vapors of selenium alloys deposited on a suitable support, and particles of photoconductive zinc oxide dispersed in resinous, film-forming binder have found wide application in the present-day document copying applications.

Since the introduction of electrophotography, a great many organic compounds have also been screened for their photoconductive properties. As a result, a very large number of organic compounds have been shown to possess some degree of photoconductivity. Many organic compounds have revealed a useful level of photoconduction and have been incorporated into photoconductive compositions.

In photoconductive insulating compositions using organic photoconductors, the photoconductor, if not polymeric, is usually carried in a film-forming binder. Typical binders are polymeric materials having fairly high dielectric strength such as phenolic resins, ketone resins, acrylic ester resins, polystyrenes and the like. A more comprehensive listing of binders appears in U.S. Pat. No. 3,755,310 (issued Aug. 28, 1973 to L. J. Rossi). The photoconductor can be dissolved with the binder to prepare a homogeneous photoconductive composition in a common solvent. In another aspect, it can be

provided as a dispersion of small particles in the binder to prepare a heterogeneous photoconductive composition. A general discussion of such dispersions and their preparation appears in U.S. Pat. No. 3,253,914 (issued May 31, 1966 to G. Schaum). There is no suggestion in the U.S. Pat. No. 3,253,914 patent of binders that are especially useful for preparing the dispersions.

Organic photoconductors demonstrate widely varying degrees of solubility in the organic solvents used to dissolve many of the common binders. In the preparation of homogeneous photoconductive insulating compositions, organic photoconductors such as p-terphenyl and others of low solubility in popular solvents cannot usually be included in sufficient concentration to provide compositions of desirable light-sensitivity. By use of dispersion techniques such as those referred to in the case of zinc oxide photoconductors, heterogeneous photoconductive insulating compositions having higher concentrations of low solubility photoconductors can be obtained, the objective being to improve light-sensitivity in the composition.

Heterogeneous organic photoconductive compositions as discussed herein can be advantageous, especially in the preparation of electrophotographic elements on which visible images will be provided. For example such elements are both lighter in weight than those having inorganic photoconductors like zinc oxide, and can be prepared to resemble bond paper. However, they have not enjoyed in such applications the popularity of photoconductive insulating compositions using inorganic photoconductors. This is largely due to the unacceptable photoconductivity of heterogeneous compositions despite their high concentrations of organic photoconductor. Homogeneous compositions of organic photoconductors, on the other hand, appear to be acceptable in their photoconductivity, but when coated on paper materials, do not have the appearance and feel of plain paper.

To improve the photoconductivity of heterogeneous photoconductive compositions having dispersed organic photoconductor particles, a variety of compounds have been studied for use as so-called chemical sensitizers or activators. When added to the photoconductive compositions it is intended that such compounds enhance the photoconductivity of the composition at least within the electromagnetic wavelength region in which the composition is intrinsically sensitive. If successful, the composition is said to be chemically sensitized or activated. Owing to the commercial popularity of homogeneous photoconductive compositions, however, the art has for the most part revealed chemical sensitizers which are specific to homogeneous compositions. In this regard, it does not generally follow that a chemical sensitizer that is useful in a homogeneous mode, is also useful in a heterogeneous mode. Similarly, as recognized in the present invention, the binder employed in a heterogeneous photoconductive insulating composition can affect not only the photoconductivity of the compositions, as pointed out in U.S. Pat. No. 3,703,372, (issued Nov. 21, 1972 to S. H. Merrill) but also can affect the ability of the composition to the chemically sensitized.

In U.S. Pat. Nos. 3,152,895 (issued Mar. 14, 1962 to G. H. Tinker et al) and 3,607,261 (issued Apr. 4, 1969 to A. B. Amidon) a variety of binders, including cellulose nitrate, are disclosed for use in photoconductive compositions comprising either inorganic or organic photoconductors. Neither of these patents, however, provide any specific teaching as to sensitization with com-

pounds of the present invention nor suggestion that ability to be sensitized may be affected by the binder employed.

Selection of a proper chemical sensitizer is further complicated by other requirements of an electrophotographic system. An element employing a chemically sensitized photoconductive composition as defined herein must, for example, readily accept and hold electrostatic charge before imagewise illumination. Often compositions employing compounds screened for use as sensitizers, although acceptably photoconductive, undesirably fail to accept a high enough charge to merit further pursuit. Compositions so failing are said to be "charge saturated". Further, though able to accept charge, compositions may be unable to hold applied charge for reasonable periods of time in the dark hence the term "dark decay".

#### SUMMARY OF THE INVENTION

Chemical sensitization of a heterogeneous photoconductive insulating composition comprising particles of an organic photoconductor dispersed in cellulose nitrate binder is provided by the use of monomeric hexachlorocyclopentenes. Compositions so sensitized readily accept electrostatic charge and substantially avoid dark decay. Preferred hexachlorocyclopentenes for use in this invention are compounds having the structure:



wherein B is



wherein

R is hydrogen or alkyl having one to four carbon atoms; R<sub>1</sub> is lower alkyl having one to four atoms, hydrogen, carboxyl, NO<sub>2</sub> or halogen; R<sub>2</sub> is —SO<sub>3</sub>H

or a metal salt thereof, —NO<sub>2</sub>, carboxyl or halogen; and R<sub>1</sub> and R<sub>2</sub> taken together are



- 10 When electrophotographic elements are prepared by applying the present photoconductive insulating dispersions to a conducting paper support, the photoconductive layer can be white and resemblant in both appearance and feel to bond paper. This is in contrast to many photoconductive papers using an inorganic species, such as a metal oxide, as the photoconductor. Further (apparently because of the particulate nature of the photoconductor, which may provide an increase in photoconductor surface) the present compositions and elements can be chemically and spectrally sensitized with low concentrations of sensitizer compounds compared to the concentrations that may be required for homogeneous compositions. This sensitization capability permits enhancement of the spectral response and electrophotographic speed of the particular photoconductor without detracting from the desired color of photoconductive compositions and electrophotographic elements described herein.
- 20
- 25
- 30
- 35

#### DETAILED DESCRIPTION OF THE PREFERRED EMBODIMENTS

- 40 The present invention provides chemical sensitization of heterogeneous photoconductive insulating compositions having particles of an organic photoconductor dispersed in a cellulose nitrate binder. To this end, monomeric hexachlorocyclopentenes are included in sensitizing amounts in the aforesaid photoconductive compositions. Within such class of sensitizers, for example, are compounds of the structure:
- 45



50 (b) 55 wherein B is either



60

(a)



(b)

65



Preferred fused carbocyclic ring-containing compounds (i.e., type (a) compounds noted above) for making microcrystalline photoconductive particles used in the present invention include naphthalene, anthracene, etc., preferably anthracene.

Preferred polyphenyl compounds, i.e., type (b) compounds noted, for making microcrystalline photoconductive particles include polyphenyl compounds of formula I above wherein the phenylene groups are para-phenylene groups. Such compounds include, for example, p-terphenyl, p-quaterphenyl, and p-sexiphenyl. Especially preferred materials are co-crystalline photoconductors comprising p-terphenyl doped with p-quaterphenyl. Techniques for making such co-crystalline photoconductors are described in copending application U.S. Serial Number 800,509 entitled CO-CRYSTALLINE PHOTOCONDUCTORS AND HETEROGENEOUS COMPOSITIONS THEREOF in the name of W. E. Yoerger filed concurrently herewith.

Preferred nitrogen-free, polyarylated photoconductors have the formula:



wherein each Ar and R<sup>1</sup>, R<sup>2</sup>, R<sup>3</sup> and R<sup>4</sup> are as described above.

Impurities in the photoconductor may affect its performance in compositions of the present type and usually samples of somewhat high purity are preferred. It will also be appreciated that photoconductors useful in the present invention, such as type (a), (b), and (c) compounds noted above, can include substituent groups, not specified herein, which do not impair image-forming properties of the photoconductor.

Table I lists representative photoconductors that are useful in the practice of this invention.

TABLE I

|                    |                                   |
|--------------------|-----------------------------------|
| Tetraphenylpyrrole | Tetraphenylethylene               |
| Anthracene         | 1,4-Diphenyl-1,3-butadiene        |
| Phenanthrene       | 1,1,4-Triphenylbutadiene          |
| Pyrene             | 1,1,4,4-Tetraphenyl-1,3-butadiene |
| p-Terphenyl        | 1,2,3,4-Tetraphenyl-1,3-butadiene |
| p-Quaterphenyl     | 1,3-butadiene                     |
| p-Sexiphenyl       | 1,6-Diphenyl-1,3,5-hexatriene     |

Sensitizers can be included in the present photoconductive insulating compositions. Useful sensitizers include spectral sensitizers, which are intended primarily to make the photoconductor light-sensitive to spectral regions not within the region of its inherent sensitivity; and chemical sensitizers (in addition to the hexachlorocyclopentenes described above) that serve primarily to increase light-sensitivity of the photoconductor in the spectral region of its inherent sensitivity as well as in those regions to which it may have been spectrally-sensitized. Spectral sensitizers can be chosen from a wide variety of materials such as pyrlyium dye salts inclusive of thiapyrlyium and selenapyrlyium dye salts such as those described in U.S. Pat. No. 3,250,615 (issued May 10, 1966 to C. C. Natali et al); the benzopyrlyium type sensitizers described in U.S. Pat. No. 3,554,745 (issued Jan. 2, 1971 to J. A. Van Allan); and defensive publication T-889,023 (published Aug. 31, 1971 to G. A. Reynolds et al); or the cyanine, merocya-

anine or azacyanine dyes described in U.S. Pat. No. 3,597,196 (issued Aug. 3, 1971 to C. J. Fox et al).

Preferred spectral sensitizers for use with the present photoconductive compositions include the benzopyrlyium dye cation 4-(thiaflavylidylmethylene)-flavylium and/or the cyanine dye cation 1,3-diethyl-2-[2-(2,3,4,5-tetraphenyl-3-pyrrolyl)vinyl]-1H-imidazo[4,5-b]quinoxalinium.

In compositions of the subject type, the present hexachlorocyclopentene sensitizers are usually included in an amount of about 0.1% to about 10% by weight of the photoconductor. Spectral sensitizers are usually present in the composition in an amount of about 0.001% to about 0.1% by weight of the photoconductor. Wider ranges can be useful. In the case of spectral sensitizers, however, unduly high concentrations can produce color that is apparent to the eye and change undesirably the appearance of compositions that are intended to provide a white background.

Matting agents are usefully included in the present photoconductive insulating compositions. A matting agent tends to avoid glossiness that might otherwise be obtained in layers prepared using the subject compositions and thereby enhance the "plain paper" appearance and feel that can characterize electrophotographic elements of this invention that use a paper support. Further, matting agents can improve the capability of such layers to receive legibly information written or otherwise marked on the layer. Matting agents are preferably electrically inert and hydrophobic, so as not to interfere with chargeability, charge retention or other parameters affecting electrophotographic imaging. Methacrylate and polyethylene beads are described in U.S. Pat. No. 3,810,759 (issued May 14, 1974 to T. H. Morse et al) as matting agents. Silicon containing materials are described as matting agents in U.S. Pat. No. 3,652,271 (issued Mar. 28, 1972 to D. M. Bornarth). An especially preferred silicon based matting agent is an inorganic oxide pigment, such as fumed silicon dioxide, that has been chemically modified to render it hydrophobic by reaction with an organic compound like a silane to substitute hydrocarbysilyl or other hydrophobic groups for the hydroxyl groups originally on the silicon dioxide chain. The fumed silica or other inorganic oxide pigment can be reacted conveniently with an appropriate silane, such as a halotrialkylsilane, merely by contact in solution. A preferred silane is chlorotrimethylsilane and incorporation of the silane in an amount of about 5 to about 15% by weight of the inorganic pigment is especially desirable. It is considered that other inorganic pigments like titanium dioxide and aluminum oxide, as well as clays, could be modified similarly by reaction with a silane to provide useful matting agents. Matting agents can be employed in a wide range of particle sizes and concentrations to provide the desired degree of surface texture. It is also well known in the art to consider the thickness of the layer comprising the matting agent when selecting matting agent of a given particle size. See, for example, the aforementioned U.S. Pat. Nos. 3,652,271 and 3,519,819 issued July 7, 1970 to E. P. Gramza et al. It should be emphasized that such matting agents can be used to advantage in a wide range of homogeneous and heterogeneous photoconductive insulating compositions.

Photoconductive insulating compositions of the present invention can be prepared merely by dispersing photoconductor having the desired particle dimensions in a solution of the cellulose nitrate binder that contains

a hexachlorocyclopentene sensitizer as described herein and also any other constituents e.g., spectral sensitizers, matting agents, etc., to be included in the composition. As mentioned elsewhere herein, the solvent for the binder should not have solvent action with respect to the photoconductor, which desirably is not dissolved or swollen in the presence of the binder solvent. After addition of the particulate photoconductor, the heterogeneous composition is usually stirred or otherwise mixed thoroughly to assure reasonable uniformity of the dispersion. As used herein, photoconductors desirably have a maximum particle diameter ranging from about 0.1 micron to about 20 microns with from about 0.1 micron to about 10 microns being preferred. If the photoconductor has not been ball-milled or otherwise processed to an appropriate particle size prior to its dispersion in the binder, a heterogeneous composition of the invention can be prepared and thereafter agitated in the presence of stainless steel balls or other agent effective to produce a milling action that causes attrition in the particle size of the photoconductor.

In the alternative, the photoconductor can be dispersed and ball-milled in a non-solvent that is a solvent for the cellulose nitrate binder and hexachlorocyclopentene of choice. Sensitizers to be included in the composition can be added to the photoconductor dispersion prior to such ball-milling. After this first ball-milling stage, the binder can be added, usually in the form of a solution. The composition is preferably again milled to obtain a uniform dispersion.

In the present compositions, the photoconductor is desirably included in an amount of at least about 40% by weight of solids in the composition and may range to 95 weight percent and higher depending on the particular application. Generally, the binder need only be present in an amount sufficient to provide adhesion between particles in the composition and between the composition and the support, if used. In various preferred embodiments, the photoconductor and any sensitizers, matte agents or other adjuvants constitute between about 70 and 90% by weight of solids in the composition, with the binder or binders making up the remainder of the composition.

As indicated above, the photoconductive insulating composition is usually prepared as a solution of the binder containing other components of the composition including dispersed photoconductive particles. In such form, the composition can be formed into a self-supporting member or it can be coated on an electrically conducting support to provide an electrophotographic element. For purposes of coating, the compositions desirably range from about 20 weight percent solids to about 40 weight percent solids. If extrusion hopper coating is to be used, the most useful solids content of the composition is usually between about 20 and 30 weight percent. For doctor blade coating, from about 30 to about 40 weight percent solids is preferred. Wider ranges may be appropriate depending on conditions of use. In preparing the compositions for purposes such as ball milling and coating, it may be desirable to use a solvent blend to provide optimal viscosity, ease of solvent removal or the like. Acetonitrile can be useful in combination with methanol to provide a solvent mixture for the cellulose nitrate binders discussed herein.

While it is preferable to use cellulose nitrate as sole binder with the hexachlorocyclopentene compounds described above, it may also be desirable to employ cellulose nitrate in combination with other insulating

resins as co-binders in the present compositions. If so desired, such other resins must be compatible with and dissolve in the solvent employed to dissolve cellulose nitrate when forming the aforesaid compositions. Furthermore, the inclusion of resins in addition to cellulose nitrate must not interfere with the ability of the described hexachlorocyclopentenes to chemically sensitize as described in accordance with the invention. Suitable other resins include, for example, conventional film-forming materials such as polyacrylics, polyesters, polyolefins and the like.

In applying the photoconductive insulating composition on a surface or support, they are usually coated by any suitable means, such as extrusion hopper, doctor blade or whirler coating apparatus, at a coverage sufficient to provide a layer of from 10 to about 25 microns thick when dry, although layers of lesser or greater thickness can be used, if desired. The dry thickness for any given wet thickness as coated will depend in part on the size of the photoconductive particles in the composition and on the amount of void volume, if any, in the layer. Coverages of from about 2 to about 15 grams per square meter of support are often used.

Suitable supporting materials on which can be coated photoconductive layers comprising the photoconductive compositions described herein include any of a wide variety of electrically conducting supports, for example, paper (at a relative humidity above 20 percent); aluminum-paper laminates; metal foils such as aluminum foil, zinc foil, etc.; metal plates, such as aluminum, copper, zinc, brass and galvanized plates; vapor deposited metal layers such as silver, nickel, aluminum, electrically conducting metals intermixed with protective inorganic oxides, such as Cr intermixed with SiO (as described in U.S. Pat. No. 3,880,657 issued Apr. 29, 1975 to A. A. Rasch) and the like coated on paper or conventional photographic film bases such as cellulose acetate, polystyrene, etc. Such conducting materials as nickel can be vacuum deposited on transparent film supports in sufficiently thin layers to allow electrophotographic elements prepared therewith to be exposed from either side of such elements. An especially useful conducting support can be prepared by coating a support material such as poly(ethylene terephthalate) with a conducting layer containing a semiconductor dispersed in a resin. Such conducting layers both with and without insulating barrier layers are described in U.S. Pat. No. 3,245,833 by Trevoy, issued Apr. 12, 1966. Likewise, a suitable conducting coating can be prepared from the sodium salt of a carboxyester lactone of maleic anhydride and a vinyl acetate polymer. Such kinds of conducting layers and methods for their optimum preparation and use are disclosed in U.S. Pat. Nos. 3,007,901 to Minsk, issued Nov. 7, 1961 and 3,262,807 by Sterman et al, issued July 26, 1966. Another useful support is paper or other fibrous material having thereon, to enhance electrical properties of the support, an electrically conducting material as described in U.S. Pat. No. 3,814,599 (issued June 4, 1974 to D. A. Cree), particularly in Columns 2 and 3 of the patent.

Photoconductive compositions according to the present invention can be employed in electrophotographic elements useful in any of the well known electrophotographic processes which require photoconductive layers. One such process is the xerographic process. In a process of this type, an electrophotographic element is held in the dark and given a blanket electrostatic charge by placing it under a corona discharge. This uniform

charge is retained by the layer because of the substantial dark insulating property of the layer, i.e., the low conductivity of the layer in the dark. The electrostatic charge formed on the surface of the photoconductive layer is then selectively dissipated from the surface of the layer by imagewise exposure to light by means of a conventional exposure operation such as, for example, by a contact printing technique, or by lens projection of an image, and the like, to thereby form a latent electrostatic image in the photoconductive layer. Exposing the surface in this manner forms a pattern of electrostatic charge by virtue of the fact that light energy striking the photoconductor causes the electrostatic charge in the light struck areas to be conducted away from the surface in proportion to the intensity of the illumination in a particular area.

The charge pattern produced by exposure is then developed or transferred to another surface and developed there, i.e., either the charge or uncharged areas rendered visible, by treatment with a medium comprising electrostatically responsive particles having optical density. The developing electrostatically responsive particles can be in the form of a dust, i.e., powder, or a pigment in a resinous carrier, i.e., toner. A preferred method of applying such toner to a latent electrostatic image for solid area development is by the use of a magnetic brush. Methods of forming and using a magnetic brush, toner applicator are described in the following U.S. Pat. Nos. 2,786,439 by Young, issued Mar. 26, 1957; 2,786,440 by Giaimo, issued Mar. 26, 1957; 2,786,441 by Young, issued Mar. 26, 1957; 2,874,063 by Greig, issued Feb. 17, 1959. Liquid development of the latent electrostatic image may also be used. In liquid development, the developing particles are carried to the image-bearing surface in an electrically insulating liquid carrier. Methods of development of this type are widely known and have been described in the patent literature, for example, U.S. Pat. No. 2,907,674 by Metcalfe, et al, issued Oct. 6, 1959. In dry developing processes, the most widely used method of obtaining a permanent record is achieved by selecting a developing particle which has as one of its components a low-melting resin. Heating the powder image then causes the resin to melt or fuse into or on the element. The powder is, therefore, caused to adhere permanently to the surface of the photoconductive layer. In other cases, a transfer of the electrostatic charge image formed on the photoconductive layer can be made to a second support such as paper which would then become the final print after development and fusing. Techniques of the type indicated are well known in the art and have been described in the literature such as in "RCA Review", Volume 15 (1954), pages 469-484.

Because the electrophotographic elements described herein can be developed in a liquid environment, as above described, the non-photoconductive surface of the element, i.e., that side of the support opposite the side carrying the photoconductive layer, can be overcoated with a so-called solvent hold-out layer. One or more of these layers serve to reduce or eliminate penetration of solvent or liquid carriers into the paper support during development. A typical hold-out layer can include pigments, pigment dispersing agents, clays, latices such as styrene-butadiene latex, polyvinylalcohol, and the like, in various proportions to give the desired result.

H and D electrical speeds to indicate the photoconductive response of electrophotographic materials such

as those discussed herein can be determined as follows: The material is electrostatically charged under, for example, a corona source until the surface potential, as measured by an electrometer probe, reaches some suitable initial value  $V_0$ , typically from 100 to about 600 volts. The charged element is then exposed to a 3000° K tungsten light source or a 5750° Xenon light source through a stepped density gray scale. The exposure causes reduction of the surface potential of the element under each step of the gray scale from its initial potential  $V_0$  to some lower potential  $V$  the exact value of which depends upon the amount of exposure in meter-candle-seconds received by the area. The results of these measurements are then plotted on a graph of surface potential  $V$  vs. log exposure for each step, thereby forming an electrical characteristic curve. The electrical or electrophotographic speed of the photoconductive composition can then be expressed in terms of the reciprocal of the exposure required to reduce the initial surface potential  $V_0$  to any fixed selected value typically  $\frac{1}{2} V_0$ . The foregoing procedure was employed in the examples below. An apparatus useful for determining the electrophotographic speeds of photoconductive compositions is described in Robinson et al, U.S. Pat. No. 3,449,658, issued June 10, 1969.

The following Examples are included to illustrate the present invention.

#### EXAMPLE 1

Photoconductive insulating compositions including 3 g. p-terphenyl, 1.07 g. cellulose nitrate (grade RS  $\frac{1}{4}$  sec supplied as 70 percent solids in isopropanol by Hercules Powder Company), 30 mg. chemical sensitizer as shown in Table I, and 12 ml. of a dye solution consisting of 0.003 g. of 4-(thiaflavylidylmethylene) flavylum chloride in 120 ml. of methanol (spectral sensitizer) were each placed in a 50 ml. vial containing 30 g. of 2.5 mm zirconium oxide milling media and milled for 2 hours by being shaken on a reciprocating paint shaker. The resultant compositions were each coated at a wet thickness of about 0.1 mm on a polyester support bearing a conducting layer of vacuum deposited nickel and dried to prepare electrophotographic elements. An otherwise identical control element without chemical sensitizer was prepared in the same manner. Each of the electrophotographic elements was charged to 300 volts (positive polarity) and thereafter exposed to a 3000° K tungsten light source for a time sufficient to discharge exposed regions to +150 volts. With the electrical speed of the control element arbitrarily designated 100, the relative speeds of the chemically sensitized elements were as shown in Table I.

TABLE I

| Chemical Sensitizer  | Relative Electrical Speed |
|----------------------|---------------------------|
| None (control)       | 100                       |
| Chlorendic anhydride | 130                       |

TABLE I-continued

|                                                                                                                                                                                                                                                     |                                                                                                                                                                                                                                                    |
|-----------------------------------------------------------------------------------------------------------------------------------------------------------------------------------------------------------------------------------------------------|----------------------------------------------------------------------------------------------------------------------------------------------------------------------------------------------------------------------------------------------------|
|                                                                                                                                                                                                                                                     |                                                                                                                                                                                                                                                    |
| $  \begin{array}{c}  \text{R}_1 \quad \text{R}_2 \\  \hline  -\text{CH}_3 \quad -\text{SO}_3\text{H} & 181 \\  -\text{H} \quad -\text{SO}_3\text{H} & 172 \\  -\text{CH}_3 \quad -\text{SO}_3\text{Ca}^{++} & 172 \\  & 2 \\  & 167  \end{array}  $ |                                                                                                                                                                                                                                                    |
|                                                                                                                                                                                                                                                     | $  \begin{array}{c}  \text{R}_1 \quad \text{R}_2 \\  \hline  -\text{NO}_2 \quad -\text{SO}_3\text{H} & 167 \\  -\text{Cl} \quad -\text{NO}_2 & 133 \\  -\text{Br} \quad -\text{Br} & 129 \\  -\text{NO}_2 \quad -\text{COOH} & 157  \end{array}  $ |

## EXAMPLE 2

Photoconductive insulating compositions including 5.7 g. anthracene (Aldrich Chemical Company, Inc. A8920-0), 2.1 g. cellulose nitrate (grade RS  $\frac{1}{4}$  sec supplied as 70 percent solids in isopropanol by Hercules Powder Company), 0.057 g. chemical sensitizer as shown in Table II, and a control composition without sensitizer, were placed in a 50 ml. vial containing 35 g. 3 mm stainless steel balls and milled for 2 hours as in example 1. The milled formulations were diluted with 9 ml. methanol and coated at a wet thickness of about 0.05 mm on a nickelized polyester support and evaluated for electrophotographic speed as in Example 1. The results were as follows:

TABLE II

| Chemical Sensitizer  | Relative Electrical Speed |
|----------------------|---------------------------|
| None                 | 100                       |
| Chlorendic anhydride | 165                       |
| Chlorendic acid      | 180                       |

Results similar to those in Tables I and II can be expected with other organic photoconductors and with other hexachlorocyclopentene sensitizers described herein.

## EXAMPLE 3

Photoconductive insulating compositions consisting of p-terphenyl photoconductor, binder, dye solution (spectral sensitizer), and hexachlorocyclopentene sensitizers of this invention were prepared, milled and coated on supports to form elements in a manner similar to the method described in Example 1. In place of cellulose nitrate, a poly(i-butylmethacrylate) binder was employed. With the electrical speed of a control element (i.e., one having no hexachlorocyclopentene sensitizer), arbitrarily assigned as 100, the results in Table III

below were obtained in determining relative electrical speed as in the preceding examples.

TABLE III

| Chemical Sensitizer  | Relative Electrical Speed |
|----------------------|---------------------------|
| None (control)       | 100                       |
| Chlorendic acid      | 100                       |
| Chlorendic anhydride | 100                       |

10 Example 3 illustrates the effect binder can play on the ability of a heterogeneous photoconductive insulating composition to be sensitized.

The invention has been described with particular 15 reference to certain preferred embodiments thereof but it will be understood that variation and modifications can be effected within the spirit and scope of the invention.

What is claimed is:

20 1. A heterogeneous photoconductive insulating composition comprising particles of an organic photoconductor chemically sensitized with a monomeric hexachlorocyclopentene and dispersed in a cellulose nitrate binder.

25 2. The composition of claim 1 wherein said photoconductor is a compound selected from the group consisting of (a) fused carbocyclic ring compounds, (b) polyphenyl compounds having the structure

30



wherein

$n$  is an integer from 1 to about 6; and (c) nitrogen-free, polyarylated compounds having the structure



wherein

$n$  is 0, 1, or 2

Ar is aryl; and

50  $R^1$ ,  $R^2$ ,  $R^3$ , and  $R^4$  individually represent hydrogen, Ar, alkyl having 1 to about 10 carbon atoms, or alkoxy having 1 to about 10 carbon atoms, with the proviso that when  $n$  is 0, both  $R^1$  and  $R^4$  are Ar, and when both  $R^1$  and  $R^4$  are hydrogen, both  $R^2$  and  $R^3$  are Ar.

3. The composition of claim 2 wherein said monomeric hexachlorocyclopentene has the structure:



wherein B is



wherein

R is hydrogen or alkyl having one to four carbon atoms;

R<sub>1</sub> is lower alkyl having one to four carbon atoms, hydrogen, NO<sub>2</sub>, halogen or carboxyl;

R<sub>2</sub> is —SO<sub>3</sub>H or a metal salt of —SO<sub>3</sub>H, NO<sub>2</sub>, halogen, or carboxyl; and R<sub>1</sub> and R<sub>2</sub> taken together are



4. The composition of claim 3 wherein B is:



and

R<sub>1</sub> is methyl or hydrogen, or carboxyl;

R<sub>2</sub> is —SO<sub>3</sub>H or a metal salt of —SO<sub>3</sub>H; and R<sub>1</sub> and R<sub>2</sub> taken together are



5. The composition of claim 2 wherein said hexachlorocyclopentene is chlorendic anhydride or chlorendic acid.

6. A heterogeneous photoconductive insulating composition comprising particles of anthracene, p-terphenyl, p-quaterphenyl, or a tetraphenylbutadiene chemi-

cally sensitized with chlorendic anhydride or chlorendic acid, and dispersed in cellulose nitrate.

7. The composition of claim 6 wherein the nitrogen content of said cellulose nitrate is from about 11.5 to about 13 percent.

8. A heterogeneous photoconductive insulating composition comprising particles of anthracene, p-terphenyl, p-quaterphenyl or a tetraphenylbutadiene dispersed in a cellulose nitrate binder and chemically sensitized with a compound having the structure

(c) 15



wherein B is

25



30

35

and R<sub>1</sub> is lower alkyl having one to four carbon atoms, hydrogen, NO<sub>2</sub>, carboxyl or halogen;

R<sub>2</sub> is —SO<sub>3</sub>H or a metal salt of —SO<sub>3</sub>H, NO<sub>2</sub>, halogen, or carboxyl; and R<sub>1</sub> and R<sub>2</sub> taken together are

45



9. The composition of claim 8 wherein the nitrogen content of said cellulose nitrate is from about 11.5 to about 13 percent.

10. The composition of claim 9 additionally comprising a matte agent and at least one cyanine or benzopyrylium spectral sensitizing dye.

11. An electrophotographic element comprising an electrically conducting support bearing a layer thereon of a photoconductive insulating composition comprising particles of an organic photoconductor chemically sensitized with a monomeric hexachlorocyclopentene and dispersed in a cellulose nitrate binder.

12. An electrophotographic element as described in claim 11 wherein said organic photoconductor is p-terphenyl and said hexachlorocyclopentene is chlorendic anhydride, chlorendic acid, or a compound having the structure:

65



wherein B is



and

R<sub>1</sub> is methyl or hydrogen, or carboxyl;  
 R<sub>2</sub> is —SO<sub>3</sub>H or a metal salt of —SO<sub>3</sub>H; and  
 R<sub>1</sub> and R<sub>2</sub> taken together are

5



13. An electrophotographic element as described in claim 12 wherein said support is an electrically conducting paper support, the nitrogen content of said cellulose nitrate is from about 11.5 to about 13 percent, and said composition additionally comprises a matte agent.

14. An electrophotographic process comprising applying a uniform charge to the surface of an electrophotographic element, imagewise exposing said charged surface to actinic radiation to form an electrostatic latent image, and developing said latent image to form a visible image, said electrophotographic element being an element as defined in claim 11.

15. An electrophotographic process comprising applying a uniform charge to the surface of an electrophotographic element, imagewise exposing said charged surface to actinic radiation to form an electrostatic latent image, and developing said latent image to form a visible image, said electrophotographic element being an element as defined in claim 13.

16. An electrophotographic copy comprising an element as defined in claim 13 and a visible image pattern on said photoconductive insulating composition layer.

\* \* \* \* \*

30

35

40

45

50

55

60

65

UNITED STATES PATENT AND TRADEMARK OFFICE  
CERTIFICATE OF CORRECTION

PATENT NO. : 4,082,550

DATED : April 4, 1978

INVENTOR(S) : William E. Yoerger

It is certified that error appears in the above-identified patent and that said Letters Patent are hereby corrected as shown below:

Column 3, line 67, after "four" insert --carbon--.

Column 7, line 66, change "2" to --12--.

Column 11, line 27, change "an" to --and--.

Signed and Sealed this

*Fifteenth Day of May 1979*

[SEAL]

*Attest:*

RUTH C. MASON  
*Attesting Officer*

DONALD W. BANNER  
*Commissioner of Patents and Trademarks*